

## UNITED STATES PATENT OFFICE

2,545,126

PROCESSING OF FATTY ACIDS AND  
MAKING GREASE THEREFROMWilliam B. Whitney, Bartlesville, Okla., assignor  
to Phillips Petroleum Company, a corporation  
of DelawareNo Drawing. Application June 7, 1948,  
Serial No. 31,595

10 Claims. (Cl. 252—39)

1

This invention relates to improved lubricants. In one of its more specific aspects, it relates to a method for improving impure saturated soaps and materials saponifiable by reaction with an alkali base for grease making. In another of its more specific aspects, it relates to a method of improving impure alkali metal or alkaline earth metal soaps of saturated fatty acids.

Lubricating greases are conventionally prepared by the combination of a suitable lubricating oil with a thickening or gelation agent by which the lubricating oil is transformed to a plastic mass. Most commonly used as such thickening or gelation agents are metal soaps of long-chain fatty acids such as those obtained from natural sources or from glyceride-yielding mixtures of fatty acids. The soaps thus prepared are dispersed in lubricating oil to form a grease.

Most naturally occurring fats and oils, or fatty acid mixtures obtained therefrom, contain appreciable amounts of unsaturated fatty acid radicals. Soaps which contain appreciable amounts of unsaturated fatty acid radicals have been conventionally used as thickening agents for greases. It has been discovered, however, that unsaturated fatty acid radicals have undesirable effects on the resulting grease because they decrease the resistance of the grease toward oxidation. Unsaturated fatty acid radicals also decrease the consistency, work stability, and water resistance of a grease.

An object of the invention is to provide an improved method for processing fatty acids for grease making. Another object is to provide an improved method for removing impurities from saturated soaps, and materials saponifiable by reaction with an alkali, for grease making. Another object is to provide an improved method for producing a lubricating grease. Another object is to provide an improved lubricating grease having improved consistency, work stability and water resistance. Other and further objects and advantages will be apparent to those skilled in the art upon study of the accompanying description and discussion.

Generally speaking, the invention resides in a method of preparing materials for grease making by processing impure saturated soaps or materials which are saponifiable by reaction with an alkali. By "materials which are saponifiable by reaction with an alkali," it is intended to include a pure unsaturated acid or ester of an unsaturated fatty acid. As pointed out above, most naturally occurring fats and oils,

5 or fatty acid mixtures obtained therefrom, contain appreciable amounts of unsaturated fatty acid radicals. Most of the undesirable impurities in saturated soaps, fatty acids, and fats generally comprise unsaturated radicals which may be converted to saturated materials or removed from the saturated materials by contacting the materials with an anhydrous alkali at a relatively high temperature, and neutralizing the mixture with a mineral acid.

10 I have found that predominantly saturated fats, fatty acids, and soaps which contain between about ten and about twenty-four carbon atoms per molecule may be greatly improved for grease making by contacting the predominantly saturated material with an anhydrous alkali, which ranges at least ten per cent by weight in excess of that stoichiometrically equivalent to the material treated, at a temperature above 20° C. The alkali or caustic material causes the fats or fatty acids to saponify. The treatment also apparently causes many of the unsaturated materials to form saturated materials. The exact reaction which takes place to cause the transformation of the unsaturated material 15 is not entirely clear. It may be that the double bond on the unsaturated material, such as oleic acid, undergoes a cis-trans isomerization, or that the unsaturated materials are converted to shorter-chain materials along with such fragments as acetic acid and oxalic acid, or that polymerization occurs, or that some combination of the above reactions takes place. I do not wish to be bound by any explanation of the processes, but only by the process which results in the improvement.

20 The excess alkali remaining after the reaction of alkali with unsaturated material is neutralized by the addition of a mineral acid as described above. The organic fatty acids are then separated from the inorganic constituents. After the separation of the fatty acids from the mixture, the fatty acids are washed with water, after which they are dried and are converted to a metal soap of the fatty acid by reacting them with a stoichiometric equivalent of an alkali. The alkali is preferably a hydroxide of an alkali metal, such as sodium or potassium, or of an alkaline earth metal, such as calcium or barium. The alkali may, however, be a carbonate of one 25 of the metals of the above classifications. The final saponification step is generally made with an aqueous alkali at a temperature below the boiling point of water.

30 35 40 45 50 55 When treating the impure saturated materials

in the presence of an alkali which is in excess of the treated materials, the stoichiometric excess may range as low as 10 per cent by weight of the treated material. It is preferred, however, that the amount of caustic be at least 25 per cent in excess of the amount stoichiometrically equivalent to the treated materials. The impure material-caustic mixture is generally heated at a temperature between about 300° C. and the scorching temperature of the treated material. It is preferred, however, to heat the mixture at a temperature between about 310° C. and 350° C. for a period of from about 15 to 45 minutes.

Selected metal salts of fatty acids having between ten and twenty-four carbon atoms per molecule and prepared in the above-described manner may be incorporated in lubricating oils, such as mineral lubricating oils or polymer oils so as to produce a highly desirable grease. It is preferred to use metal salts of fatty acids which have a carbon content of from fourteen to twenty carbon atoms per molecule. Generally between 5 and 65 per cent by weight of a metal salt of a fatty acid, prepared as above described, may be incorporated in the lubricating oil at a temperature of between about 50° C. and 250° C. It is preferred, however, to incorporate between 15 and 50 per cent by weight of an improved saturated soap, prepared by the method of the instant invention, in a selected lubricating oil. Such a mixture of a properly selected metal salt and a lubricating oil will, when cooled, preferably at a rapid rate, form a gel.

After the improved, saturated, high molecular weight fatty acids have been resaponified to form metal soaps of the fatty acid, the soap may be dispersed in a mineral oil by heating to a temperature at which the soap begins to ball in the oil during the stirring. The balling will usually begin to occur in the vicinity of 170° C. It is not, however, preferred to cool the mixture from that point because of the difficulty in working to form a grease of even texture. The soap-lubricating oil mixture is preferably heated to a point where complete dispersion of the soap in oil is effected. It is then preferred to cool the soap-oil mixture at a rapid rate so as to produce a gel. The temperature below which the grease should be cooled is that at which solidification from a liquid to a gel occurs. This temperature is definite and possibly related to the crystalline or colloidal structure of the metal salt, or at least it is a characteristic of the soap-oil mixture. It is not intended that the temperature to which the mixture is cooled should be limited to any specified temperature so long as it is below the gelation temperature. It is desired, however, that the time of cooling be as short as possible, generally within a period of from 10 to 600 seconds. Longer periods of time may be used for cooling these mixtures if desired, but it is preferred to cool the heated mixture to a gel within a period of from 10 to 300 seconds. The cooled grease may be worked to obtain the desired consistency.

When a soap is to be treated in accordance with this invention, it is usually preferable to treat the soap with an alkali derived from the same metal as the soap. Sodium, potassium, calcium, and barium salts of fatty acids processed in the manner above described are among those salts which may be utilized to form desirable greases of this invention. Other metal salts may, however, be utilized to advantage in the preparation of such greases.

The advantages of preparing the metal salts by

the method of this invention are even more apparent upon examination of the following examples. The specific reactants and specific conditions of reaction are presented as being typical and should not be construed to limit the invention unduly.

#### EXAMPLE I

Sodium stearate containing as an impurity a substantially equal amount of sodium oleate was treated with a quantity of alcoholic sodium hydroxide solution such that, on evaporation of the solvent, the mol ratio of sodium stearate to impurity to sodium hydroxide was approximately 1:1:1.5. The alcoholic solution of sodium hydroxide was used to obtain uniform distribution of the hydroxide and permit easy removal of the solvent.

The mixture was dried and then heated to between 310° C. and 320° C. for a period of about 20 minutes. The mixture was then cooled and was acidified with hydrochloric acid. The fatty acid was recovered and was washed with water, after which it was reacted with sodium hydroxide so as to resaponify the fatty acid. Twenty per cent by weight of the resulting sodium soap was dispersed in 80 per cent by weight of a lubricating oil, the properties of which are shown in Table II below. The dispersion of the soap in the lubricating oil was accomplished by heating the mixture to about 220° C. and cooling rapidly. The resulting mass was worked in an A. S. T. M. grease worker (Precision Scientific Motormatic Model) as described in A. S. T. M. test D-217-44T. The consistency and work stability of the resulting grease is set forth below in Table I as grease A.

#### EXAMPLE II

A portion of sodium stearate soap which was identical with the original soap in Example I was converted to a grease by dispersing 20 per cent by weight in a fraction of the lubricating oil used in Example I, the oil making up 80 per cent by weight of the soap-oil mixture. The mixture was heated to about 220° C. and cooled rapidly. The resulting mass was worked in the A. S. T. M. grease worker described in Example I. The results of the test made in the grease worker are recorded in Table I below for grease B.

#### EXAMPLE III

A sodium stearate soap fraction identical with that used in Example II and to the original soap of Example I was treated with a quantity of aqueous sodium hydroxide solution (25 per cent concentration) in a quantity sufficient that in the final mixture 1.5 moles of the sodium hydroxide were present for each mol of fatty acid salt. The soap-alkali mixture was then heated at 110° C. for about 30 minutes with constant stirring. The mixture was neutralized with hydrochloric acid, and, on cooling, free fatty acids were removed. The solidified free fatty acids were liquefied by heating, after which they were washed with water and subsequently cooled. The solidified fatty acids were removed and dissolved in isopropyl alcohol, neutralized with sodium hydroxide, and evaporated to dryness. Twenty per cent by weight of the soap formed was dispersed in a fraction of the lubricating oil used in Examples I and II. After heating and rapid cooling, the resulting gel was worked in the A. S. T. M. grease worker described above. The results of the test in the grease worker are shown below in Table I for grease C. The unworked gel resulting after

rapid cooling was firm and clear, but worked to a granular mass which did not become quite smooth before the grease softened to such an extent that it exceeded the dial reading of the micro penetrometer.

tween ten and twenty-four carbon atoms per molecule and containing as an impurity an unsaturated material selected from the group consisting of fats, fatty acids, and soaps of fatty acids, in the presence of an excess of an anhy-

TABLE I  
*Comparison of stability of greases on working*

| Soap Derived from                                  | M. P. of<br>Free Acid<br>Mixture,<br>°C. | Micropenetration on Working, Strokes |      |       |       |        |        |         |
|----------------------------------------------------|------------------------------------------|--------------------------------------|------|-------|-------|--------|--------|---------|
|                                                    |                                          | 60                                   | 1000 | 2000  | 5000  | 10,000 | 50,000 | 100,000 |
| Grease B Untreated, impure stearate                | 45                                       | -----                                | 336  | ----- | 365   | 385    | -----  | -----   |
| Grease A Stearate treated with anhydrous hydroxide | 47                                       | -----                                | 176  | ----- | 202   | 248    | -----  | 375     |
| Grease C Stearate treated with aqueous hydroxide   | 108                                      | 248                                  | 280  | 393   | ----- | -----  | -----  | -----   |

TABLE II  
*Physical constants of oil used in preparing grease*

| Vis. SUS<br>100 F. | Vis. SUS<br>210 F. | VI   | $n^{20}$ | $D_4^{20}$ |
|--------------------|--------------------|------|----------|------------|
| 183.2              | 44.6               | 90.7 | 1.4748   | .8690      |

Comparison of the micropenetration readings resulting from the tests made with the greases of Examples I, II, and III clearly shows that the grease formed from the fatty acid which was treated with the anhydrous sodium hydroxide had far greater consistency than either of the other two greases.

As will be evident to those skilled in the art, various modifications can be made in the selection of the solvent for the base solution used in treating the soap or the materials which are saponifiable by treatment with a base solution. It is preferred, however, that the selected alkali or base have a similar basicity to the base of the soap treated. Other modifications may be made in the oil used as the dispersion agent for the production of a grease. It is believed that various other modifications of this invention can be made or followed in the light of the foregoing disclosure and discussion without departing from the spirit or scope of the disclosure or from the scope of the claims.

I claim:

1. An improved method for making grease which comprises the steps of improving at least one material selected from a group of saturates consisting of fats, fatty acids, and soaps of fatty acids, which saturates contain as impurities unsaturates of a chemical type similar to said saturates, by heating at least one of said saturates having between ten and twenty-four carbon atoms per molecule in the presence of an excess of an anhydrous alkali at a temperature between 300° C. and the scorching temperature of the saturate material for between 15 and 45 minutes, whereby said unsaturates are decomposed and saponifiable materials are saponified; reacting resulting soap with a mineral acid to liberate free organic acids; recovering organic acid materials from said resulting mixture; washing said organic acid materials; resaponifying said organic acid materials by heating with a stoichiometric amount of a metal base; incorporating resulting soap in oil by heating and rapidly cooling the soap-oil mixture to form a gel.

2. A method of producing an improved grease which comprises the steps of heating at least one saturated soap of a fatty acid having be-

drous alkali at a temperature between 300° C. and the scorching temperature of the treated material for between 15 and 45 minutes, whereby said unsaturate material is decomposed and any saponifiable materials are saponified; reacting the resulting soap with a mineral acid to liberate free organic acids; recovering organic acid materials from the resulting mixture; washing said organic materials; resaponifying said organic acid materials by heating with a stoichiometric amount of a metal base to form a soap; incorporating between 5 and 65 per cent by weight of said soap in between 35 and 95 per cent by weight of a lubricating oil at a temperature of between 170° C. and 250° C.; cooling said soap in an oil mixture to form a gel within a period of from 10 to 600 seconds; and working said gel to the desired consistency.

3. The method of claim 2, wherein said metal base is derived from the same metal as said saturated soap.

4. A method of producing an improved grease which comprises the steps of heating at least one saturated fatty acid having between ten and twenty-four carbon atoms per molecule and containing as an impurity at least one unsaturated material selected from the group consisting of fats, fatty acids, and soaps of fatty acids, in the presence of an excess of an anhydrous alkali at a temperature between 300° C. and the scorching temperature of the treated material for between 15 and 45 minutes, whereby said unsaturated material is decomposed and any saponifiable materials are saponified; reacting the resulting soap with a mineral acid to liberate free organic acids, recovering organic acid materials from the resulting mixture; washing said organic materials; resaponifying said organic acid materials by heating with a stoichiometric amount of a metal base to form a soap; incorporating between 5 and 65 per cent by weight of said soap in between 35 and 95 per cent by weight of a lubricating oil at a temperature of between 170° C. and 250° C.; cooling said soap in an oil mixture to form a gel within a period of from 10 to 600 seconds; and working said gel to the desired consistency.

5. A method of producing an improved grease which comprises the steps of heating at least one saturated fat having between ten and twenty-four carbon atoms per molecule and containing as impurities at least one unsaturated material selected from the group consisting of fats, fatty acids, and soaps of fatty acids, in the presence of an excess of an anhydrous alkali at a temperature between 300° C. and the scorching temperature of the treated material for between 15 and 45

minutes; whereby said unsaturate material is decomposed and any saponifiable materials are saponified; reacting the resulting soap with a mineral acid to liberate free organic acids; recovering organic acid materials from the resulting mixture; washing said organic materials; resaponifying said organic acid materials by heating with a stoichiometric amount of a metal base to form a soap; incorporating between 5 and 65 per cent by weight of said soap in between 35 and 95 per cent by weight of a lubricating oil at a temperature of between 170° C. and 250° C.; cooling said soap in an oil mixture to form a gel within a period of from 10 to 600 seconds; and working said gel to the desired consistency.

6. A method of producing an improved grease which comprises the steps of heating at least one saturated material having between ten and twenty-four carbon atoms per molecule which saturated material is selected from the group consisting of fats, fatty acids, and soaps of fatty acids and containing as an impurity therein at least one unsaturated material selected from the group consisting of fats, fatty acids, and soaps of fatty acids, in the presence of an excess of an anhydrous alkali at a temperature between 300° C. and the scorching temperature of the treated material for between 15 and 45 minutes, whereby unsaturate materials are decomposed and any saponifiable materials are saponified; reacting the resulting soap with a mineral acid to liberate free organic acids; recovering organic acid materials from the resulting mixture; washing said organic materials; resaponifying said organic acid materials by heating with a stoichiometric amount of a metal base to form a soap; incorporating between 5 and 65 per cent by weight of said soap in between 35 and 95 per cent by weight of said lubricating oil at a temperature of between 50° C. and 250° C.; cooling said soap-oil mixture to form a gel within a period of from 10 to 600 seconds; and working said gel to the desired consistency.

7. A method of producing an improved grease which comprises the steps of heating at least one saturated material having between ten and twenty-four carbon atoms per molecule which saturated material is selected from the group consisting of fats, fatty acids, and soaps of fatty acids and containing as an impurity therein at least one unsaturated material selected from the

group consisting of fats, fatty acids, and soaps of fatty acids, in the presence of an excess of an anhydrous alkali at a temperature between 300° C. and the scorching temperature of the treated material for between 15 and 45 minutes, whereby unsaturate materials are decomposed and any saponifiable materials are saponified; reacting the resulting soap with a mineral acid to liberate free organic acids; recovering organic acid materials from the resulting mixture; washing said organic materials; resaponifying said organic acid materials by heating with a stoichiometric amount of a metal base to form a soap; incorporating between 15 and 50 per cent by weight of said soap in between 50 and 85 per cent by weight of said lubricating oil at a temperature between 50° C. and 250° C.; cooling said soap-oil mixture to form a gel within a period of from 10 to 300 seconds; and working said gel to the desired consistency.

8. The method of claim 6, wherein said saturated material is a sodium soap; said alkali-soap mixture is heated at a temperature between 310° C. and 350° C. and said metal base is an aqueous solution of sodium hydroxide.

9. The method of claim 6, wherein said saturated material is a potassium soap; and said alkali-soap mixture is heated at a temperature between 310° C. and 350° C.

10. The method of claim 6, wherein said saturated material is a calcium soap; and said alkali-soap mixture is heated at a temperature between 310° C. and 350° C.

WILLIAM B. WHITNEY.

#### REFERENCES CITED.

The following references are of record in the file of this patent:

#### UNITED STATES PATENTS

| Number    | Name           | Date           |
|-----------|----------------|----------------|
| 1,429,114 | Stiepel        | Sept. 12, 1922 |
| 1,598,225 | Walker         | Aug. 31, 1926  |
| 1,973,537 | Miller et al.  | Sept. 11, 1934 |
| 2,070,014 | Lincoln et al. | Feb. 9, 1937   |
| 2,428,123 | Morgan et al.  | Sept. 30, 1947 |

#### OTHER REFERENCES

Spitzer et al.: Conjugation of Drying Oil Fatty Acids, reprint of articles in American Paint Journal, December 15 and 22, 1941, page 1.